

No. 830,208.

PATENTED SEPT. 4, 1906.

E. A. COLBY.

CRUCIBLE.

APPLICATION FILED NOV. 23, 1905.



Fig. 1.



Fig. 2.



Fig. 3.



Fig. 4.



Fig. 5.



Fig. 6.

WITNESSES:

Park Benjamin Jr  
Entwistle, Boston.

INVENTOR

Edward A. Colby  
BY  
Park Benjamin  
His ATTORNEY

# UNITED STATES PATENT OFFICE.

EDWARD A. COLBY, OF NEWARK, NEW JERSEY.

## CRUCIBLE.

No. 830,208.

Specification of Letters Patent.

Patented Sept. 4, 1906.

Application filed November 23, 1905, Serial No. 288,636.

*To all whom it may concern:*

Be it known that I, EDWARD A. COLBY, a citizen of the United States, residing at Newark, in the county of Essex and State of New Jersey, have invented a certain new and useful Improvement in Crucibles, of which the following is a specification.

The invention relates to a crucible for use in an electrical-induction furnace wherein the charge in said crucible is melted by currents induced therein as a secondary circuit from a primary circuit in suitable proximity.

The invention consists in the construction of the crucible in annular form having the chamber-surface of one wall frusto-conical, also in a crucible-lining of refractory material adapted to become crushed by the compressive strain of the material solidifying in said crucible.

20 The object of the invention is, first, to enlarge the crucible-opening, and so render it more easily charged and the solidified material more easily extracted than if the walls were truly cylindrical, and, second, to protect the crucible-wall from rupture or cracking due to the strains due to the solidifying mass therein.

In the accompanying drawings, Figure 1 is a transverse section of a crucible embodying my invention. Fig. 2 is a similar section 30 of a modified form thereof. Fig. 3 shows, on a smaller scale, an annular lining of friable material separate from the crucible shown in Fig. 1 and adapted to fit therein. Fig. 4 shows a similar lining adapted to 35 the crucible shown in Fig. 2. Figs. 5 and 6 show lining-sections, of which the linings of Figs. 3 and 4 may, if desired, be composed.

Similar letters of reference indicate like parts.

40 The crucible is made of any suitable refractory material molded into form in the usual way. As shown in Fig. 1, the chamber-surface A of the outer wall B is a right cylinder. The chamber-surface C of the inner wall D is frusto-conical.

In order to protect the crucible from rupture, I apply to the surface C a lining E of any refractory material which is more friable and hence more easily crushed than the solid

50 refractory material of the crucible itself, or which even if of the same refractory material as said crucible is in any suitable way made less dense or less resistant to the compressive strain due to solidifying metal in said crucible than an equal thickness of the

refractory material of said crucible itself would be. Said lining may be originally in annular form, as shown in Figs. 3 and 4, and simply inserted in place, or it may be composed of sections, as shown in Figs. 5 and 6, or it may be applied in a plastic state and left to harden before use. It is of course to be understood that the specific material or compound of materials selected for the lining shall not be of a nature chemically to combine with the molten charge in the crucible to produce a detrimental effect therein.

In the modification shown in Fig. 2 the chamber-surface A of the outer wall B is inverted frusto-conical, while the chamber-surface C of the inner wall D is a right cylinder. The lining E, as before, is applied to the surface C

I claim—

1. A refractory crucible-lining constructed to yield to the compressive strain of solidifying metal.

2. A refractory lining for annular crucibles formed of friable material constructed to yield to the compressive strain of solidifying metal.

3. In combination with a crucible of refractory material, a refractory lining less resistant to internal pressure than the wall of said crucible to which it is applied.

4. In combination with a crucible of refractory material, a refractory lining molded into form to fit said crucible and less resistant to internal pressure than the walls of said crucible to which it is applied.

5. In combination with a crucible of refractory material, a refractory lining constructed in sections to fit said crucible and less resistant to internal pressure than the wall of said crucible to which it is supplied.

6. A lining for annular crucibles formed in sections of friable refractory material constructed to yield to the compressive strain of solidifying metal.

7. In combination with an annular crucible of refractory material, and on the chamber-surface of the inner wall thereof a refractory lining of material less resistant to internal pressure than the wall of said cylinder.

In testimony whereof I have affixed my signature in presence of two witnesses.

EDWARD A. COLBY.

Witnesses:

PARK BENJAMIN, Jr.,  
Wm. H. SIEGMAN.